

Apr. 17, 1923.

1,452,275

W. G. HOUSKEEPER

METHOD OF MAKING LEADING-IN CONDUCTORS

Filed Feb. 27, 1920

Fig. 1.



Fig. 2.



Fig. 3.



Inventor:

William G. Houskeeper.

by Jas Ch. Paunes Atty.

## UNITED STATES PATENT OFFICE.

WILLIAM G. HOUSKEEPER, OF NEW YORK, N. Y., ASSIGNOR TO WESTERN ELECTRIC COMPANY, INCORPORATED, OF NEW YORK, N. Y., A CORPORATION OF NEW YORK.

## METHOD OF MAKING LEADING-IN CONDUCTORS.

Continuation of application Serial No. 158,574, filed March 30, 1917. This application filed February 27, 1920. Serial No. 361,706.

*To all whom it may concern:*

Be it known that I, WILLIAM G. Hous-  
keeper, a citizen of the United States, re-  
siding at New York, in the county of New  
5 York and State of New York, have invented  
certain new and useful Improvements in  
Methods of Making Leading-In Conductors,  
of which the following is a full, clear, con-  
cise, and exact description.

10 This invention is a continuation of ap-  
plication, Serial No. 158,574 filed March 30,  
1917 and relates to leading-in conductors  
for incandescent lamps, mercury arc recti-  
fiers, vacuum tubes, and the like, and more  
15 particularly to those which are made from  
one or more of the base metals.

Extreme care has heretofore been con-  
sidered necessary in sealing in base leading-  
in conductors, to secure a seal which, under  
20 the conditions of operation, will prove satis-  
factory. A seal constructed without atten-  
tion being paid to the difference in coeffi-  
cients of expansion of the materials used  
25 is incapable of preventing air from passing  
into an evacuated bulb or a sealed inert gas  
from escaping out into the atmosphere. It  
is common knowledge that the difficulty thus  
experienced has been obviated by the use  
30 of so-called fluxing material. When the  
latter is used there appears to be an ab-  
sorption of any oxide which may have  
formed on the surface of the conductor, or  
in some cases actual welding of the flux to  
35 the surface of the conductor. Such flux  
is usually chosen so that a perfect union may  
be had with the glass or other vitreous ma-  
terial of the evacuated bulb.

As the use of a flux, however, is unde-  
sirable, inasmuch as it adds to the expense  
40 involved by requiring an additional opera-  
tion, attempts have been made to make  
a satisfactory seal without using a fluxing  
material. In practically every case, how-  
ever, it has been found that great care must  
45 be exercised in preventing the formation of  
oxide on the surface of the conductor. At-  
tenuated and looped parts have been sealed  
into vitreous materials which appear, on  
experimentation, to withstand the heating  
50 and cooling of the seal without exhibiting  
any leaks. The manufacture on a commer-  
cial scale of such seals, however, is pro-  
hibitive on account of the failure of a large  
proportion due to traces of oxide on the

surface of the conductor. Moreover, a lead-  
55 ing-in conductor made in this way is ex-  
tremely weak mechanically, and has proven  
to be too fragile for commercial use.

An object of this invention is to provide  
a method by which base leading-in con-  
ductors may be sealed in glass or other vit-  
reous material without the use of a flux  
or without the exercise of care to prevent  
oxidation on the surface of said conductor.

Another object is to so shape that portion  
60 of the leading-in conductor which is re-  
tained in the vitreous material that the above  
may be accomplished without necessitating  
a reduction in cross section of said con-  
ductor.

70 It has been found that a very satisfactory  
seal may be made if due consideration is  
given to the strains and stresses which are  
present in the composite structure formed  
by imbedding a metallic conductor in glass  
75 or other vitreous material. While the in-  
vention herein may be readily carried out  
when copper, silver, brass, iron, nickel, or  
any other conducting material having a dif-  
ferent coefficient of expansion from that of  
80 the glass or other vitreous material into  
which it is to be sealed, is used, the use of  
copper in this connection will be more par-  
ticularly referred to herein.

When a copper conductor is sealed into  
85 glass, there is a tendency on cooling, for  
the copper to shrink faster than the glass  
wall. This is due to the different coefficients  
of expansion possessed by these two ma-  
terials. When this shrinking takes place the  
90 copper and glass may become wholly sep-  
arated or the glass may become disrupted,  
or both. When this occurs, a direct com-  
munication between the inside of the recep-  
tacle and the outer atmosphere is estab-  
95 lished. If the conductor is made in a rib-  
bon form the cracks will tend to form on  
the edges of the ribbon. The thicker the  
ribbon in comparison with its width, and  
the thicker the glass wall surrounding the  
100 ribbon at the seal, the easier it will be for  
the cracking to take place. When a flux  
medium is used in sealing-in operations,  
rupture of the seal is prevented, because the  
stresses in the structure are less, probably  
105 due to the lower temperature at which the  
flux medium solidifies. Without the flux,  
however, it is apparent from experiments

that unless some specific design of that part of the conductor which remains in the glass is secured, no permanent seal can be made.

It has been found that if the width of the ribbon employed is several times its thickness, and if the edges of the ribbon are sharpened, making the angles formed at the edges very small; the glass and copper yield slightly when the cooling of the seal takes place and the engagement of their surfaces is not broken. When the width of the ribbon is made large in comparison with its thickness, the glass wall yields slightly and follows the shrinking in the thickness of the ribbon; and when the edges of the ribbon are sharpened, the glass wall is enabled to grip the ribbon with a sufficient firmness to resist the tendency of the latter to shrink away from the glass wall at the edges of the ribbon.

Thus a seal may readily be made without the addition of a flux, or without exercising special care to prevent oxidation on the surface of the conductor.

25 In the drawings, Fig. 1 is an elevation of a portion of a container having a ribbon of contacting material sealed into the wall thereof; Fig. 2 is a view of the same structure taken at a right angle to the view of Fig. 1; and Fig. 3 is a cross-sectional view on a larger scale taken on the line 3, 3 of Fig. 1.

Referring to the drawings, a conductor of copper in the form of a ribbon 4 is shown sealed at 5 into the wall of the container which is shown in the form of a tube 6 of glass. At the point where the ribbon 4 is sealed into the glass, the edges of said ribbon are sharpened as shown. This sharpening may be done in any suitable manner, as, for example, by filing off diagonally opposite corners on the edges of the ribbon. This filing should be so done that no pronounced corner is left; that is, so that the filed surface and the original surface of the ribbon run smoothly into one another. The sharpened edges of the ribbon should be not more than .0015 of an inch thick and thinner if they can conveniently be so made. Furthermore the angle at which the surfaces meet should be small; for example, not more than 8°. It is also desirable that the ratio of the width of the ribbon to its thickness should be comparatively large; for example, ten or more.

If metals other than copper be used, the edge angles alone will have to be varied. Thus, for example, if iron be employed, the edge angles should be not greater than 4°.

60 In producing a seal according to the preferred method, the conductor is held in a glass-worker's fire having an oxidizing flame. The conductor is moved about in the fire until each portion of the part to be sealed in has been heated to a good, red heat. This op-

eration will require on an overage from four to six seconds when an eight-burner fire is used. The heat covers the copper with a thin hard coating of oxide and prevents the subsequent escape of occluded gases from the copper during the sealing-in process. The copper ribbon is then introduced into the glass and both are heated to a good, yellow heat when the glass is pressed firmly against the copper with glass-workers' pliers.

75 While the above has been found to be the best method of sealing in the conductor free from flux and in the presence of oxide, there are other ways in which the operation could be carried out. For example, it is not necessary that the ribbon be completely covered with the oxide of copper before it is sealed into the glass. As a matter of fact the seal could be made satisfactorily if care were taken to prevent all oxidation. Although 80 the present invention is herein described as particularly useful in connection with the so-called leading-in conductors, it will be understood that it is not confined to that particular use but may be employed in connection with 85 so-called "anchor wires" or other structures which it is necessary to imbed in vitreous material such as glass.

What is claimed is:

1. The method of making a seal between a 90 metallic conductor and a vitreous material which consists in shaping the conductor into a ribbon form, having a width at least ten times its thickness, edge angles of not more than 8 degrees, and imbedding said ribbon 100 in the glass without the addition of a flux thereto.

2. The method of making a seal between glass and copper which consists in shaping the copper into a ribbon form, having a width at least ten times its thickness, edge angles of not more than eight degrees, and imbedding said ribbon in the glass without 105 the addition of a flux thereto.

3. The method of making a seal between copper and glass, which consists in shaping the copper into a ribbon form having a width at least ten times its thickness and edge angles of not more than eight degrees, oxidizing said ribbon and imbedding it in 115 said glass without the addition of a flux thereto.

4. The method of making a seal between a metallic conductor and a vitreous material which consists in shaping the conductor into a ribbon form having a width at least ten times its thickness, heating the conductor until its surface is covered with oxide and then embedding it in such vitreous material without the addition of a flux thereto.

5. The method of making a seal between a metallic conductor and a vitreous material which consists in shaping the conductor into a ribbon form having a width at least ten times its thickness and edge angles of not 130

more than eight degrees, heating the conductor until its surface is covered with oxide, and then embedding it in such vitreous material without the addition of a flux thereto.

5 6. The method of making a seal between a metallic conductor and a vitreous material which consists in shaping the conductor into

ribbon form, tapering it to narrow angles at each edge and embedding in vitreous material without the addition of a flux thereto. 10

In witness whereof, I hereunto subscribe my name this 25th day of February, A. D. 1920.

WILLIAM G. HOUSKEEPER.